

## UNITED STATES PATENT OFFICE

PAUL H. ROGERS, OF HARTSVILLE, SOUTH CAROLINA

## MANUFACTURE OF PAPER-BOARD

No Drawing.

Application filed September 2, 1931. Serial No. 560,865.

This invention has reference to the manufacture of paper or paper-board and more particularly to the corrugated sheet forming one member of the two-ply or three-ply sheets now widely used for a variety of purposes and known as "box board"; but the invention is not restricted to that use.

Heretofore the corrugated sheet of box board has been most commonly made from straw-board, which has the necessary or desirable qualities when the weight of the sheet, at the standard thickness of 0.009 of an inch, is from 32 to 34 pounds per thousand square feet.

In view of the uses to which corrugated paper-board is put, it is very desirable to reduce the weight thereof if that can be done without loss in respect of other essential characteristics.

It has been attempted, therefore, to produce a paper-board suitable for corrugating (known in the trade as "corrugating board"), that is to say, a paper-board having the properties of rigidity, lightness and running well in the corrugating machine by using a pulp made of a wood fiber (pine wood pulp) which is substantially lighter than that from which the commercial corrugated straw-board is made; but it has been found that the gain in lightness was at the expense of some of the essential or desirable properties of the finished corrugated sheet.

Use has also been made, in the manufacture of corrugating board, of pulp obtained by the semi-chemical process from chestnut chips. This product has been found satisfactory as regards strength and other properties when the weight is approximately 34 pounds per 1000 square feet; but this material cannot be used for the specified purpose at a substantially less weight without loss in respect to rigidity and bending quality.

One of the leading objects of the present invention is to produce a paper stock suitable for making corrugating board which, at the standard thickness, will have a weight substantially less than that of a sheet made from the pulp last referred to, or made of straw-board, without sacrificing any of the essential or desirable properties thereof.

Another object of the invention is to produce, at relatively low cost, corrugating board which, while having a minimum weight at the standard thickness, possesses improved characteristics in respect to bending and resistant properties and in respect to its capacity for quickly absorbing the glue whereby the corrugated sheet is attached to the other sheets (or sheet) of the commercial fabric.

The foregoing and other objects of the invention are attained by the admixture with semi-chemical pulp, known as neutral sulphite pulp, a product developed by the U. S. Forest Products Laboratory, of a certain proportion of cotton fibers, such as linters or hull fibers. The cotton fibers may be used to good advantage in a raw state, thereby saving the cost of cooking or treating. The term "cotton fibers" is used herein in a generic sense embracing linters and hull fibers.

The preferred proportions of the mixture are 75 to 90 percent of semi-chemical pulp and 10 to 25 percent of cotton fibers by weight.

The mixture is preferably made in the beating engine, but may be effected at any convenient stage of the process of manufacture and by any appropriate means. Any approved make of beating engine, such as the Hollander, may be used.

One advantageous result of the invention is that it permits the utilization of the hull fibers of the cotton seed, thereby effecting a substantial saving in cost. These low cost hull fibers may be used without any preliminary treatment for cleansing or other purpose.

It is not necessary for the purposes of this invention that the fibers be separated entirely from the hulls; as the hulls with attached fibers may be chemically digested and in that state admixed with the semi-chemical or other standard pulp.

As already stated, the principal advantage resulting from the addition of cotton fibers to the semi-chemical pulp is a substantial reduction in the weight of the product without impairing its other desirable characteristics, but rather with an improvement

therein. Thus, by the use of the proportion of cotton fiber stated above, the weight of the sheet of standard thickness (0.009") may be reduced one fourth or more. That is, instead of running from 32 to 34 pounds per 1000 square feet, its weight may be reduced to from 24 to 26 pounds per 1000 square feet or even less. And since the price is based upon the area of the sheet and not upon its weight, the gain in the value of the product per ton is substantial.

10 I have found that in paper board made of semi-chemical or neutral sulphite pulp and cotton fibers (linters or hull fibers) the semi-chemical pulp imparts in ample degree the required rigidity, which is of prime importance in corrugating board, that is, the capacity to maintain the corrugated form, to withstand pressure and to absorb shocks; while the cotton linters or hull fibers furnish the requisite bulk and also impart to the pulp the necessary bending quality, that is, the capacity to run well on the corrugating machines and to take readily the impress of the corrugating devices. I have found that cotton hull fibers (a product only recently made available) impart to any standard pulp a very superior running quality.

15 30 Furthermore, since the hull fibers cost less per pound than the semi-chemical pulp, the cost of the aggregate is reduced in proportion to the percentage of hull fibers in the mixture.

35 What is claimed is:—

1. Corrugating paper-board composed of semi-chemical pulp having in admixture therewith cotton fibers.
2. Corrugating paper-board composed of semi-chemical pulp having in admixture therewith cotton fibers in the proportion of from about ten to about twenty-five percent of the mass by weight.
3. Corrugating paper-board composed of semi-chemical pulp having in admixture therewith cotton fibers in the proportion of about ten percent of the mass by weight.

40 45 In testimony whereof I have signed this specification.

50 PAUL H. ROGERS.

55

60

65